

May 4, 1926.

1,583,248

P. H. G. DURVILLE

PROCESS FOR BOTTOM CASTING

Filed March 14, 1922

Fig.1



Fig.2



Fig.3



Fig.6



Fig.5



Fig.7



Fig.8



Inventor

Pierre H. G. Durville

By Edward C. Sarnett  
Attorney.

Patented May 4, 1926.

## UNITED STATES PATENT OFFICE.

PIERRE HENRI GASTON DURVILLE, OF PARIS, FRANCE.

## PROCESS FOR BOTTOM CASTING.

Application filed March 14, 1922. Serial No. 543,731.

*To all whom it may concern:*

Be it known that I, PIERRE HENRI GASTON DURVILLE, citizen of the Republic of France, residing at 65 Rue d'Amsterdam, Paris, Seine, France, have invented certain new and useful Improvements in or Relating to a Process for Bottom Casting, of which the following is a specification, reference being had therein to the accompanying drawing.

10 It is recognized that one of the most favorable conditions for the production of very sound ingots and mouldings is that whereby the filling of ingot moulds or metal or sand moulds is effected while causing during the operation the least possible agitation of the molten metal.

This condition is not at all events attained by a direct pouring into the molds, where considerable agitation of the metal flowing into the metal already cast inevitably occurs and causes a very large amount of oxide, flows, slag, dross and pellicular folds a considerable portion of which elements remain imprisoned in the casting even after a portion has risen in the dead heads reserved for the purpose. This condition, moreover, is not attained in current operations as hitherto practised in bottom casting by providing a lateral duct to the mould or by reserving 30 an analogous conduit in the sand of the sand mould.

In fact, if the section of the metal inlet orifice at the bottom of the mould is reduced in comparison with that of the charging or feeding orifice of the lateral conduit in a manner to maintain the latter full immediately after the commencement of the pouring, the hydrostatic pressure corresponding to the height of the conduit causes a gushing 40 at the bottom of the mould much more like a jet of water as like a fountain which occasions a prejudicial agitation and disturbance of the liquid.

But if, on the contrary, the inlet section at the base of the mould is greater than that of the charging orifice of the lateral conduit, the latter cannot be kept to the full level during the whole period of the casting and the height of the fall of the molten metal 50 into the conduit, a height at the commencement equal to that of the mould, necessarily induces a prejudicial agitation.

Within the limits of this dilemma, it has not been possible to find an appropriate middle course, although the ordinary bottom casting device never gives results sufficiently

satisfactory to compensate the complication which it involves. Also, in spite of the well-known advantages appertaining to top casting of objects of large dimensions, the actual insufficiency of the casting processes always limits the adoption of this means.

Various processes of filling by rotating and tipping have been employed with success for remedying the inconveniences that occur in the two current modes of casting by maintaining during the continuance of the operation to a tranquil filling of the moulds, avoiding disturbances and the consequent defects, but owing to the tipping these latter methods, by at least necessitating the handling of large masses, are particularly convenient only for the production of small and medium sized units.

The present invention has for its object and its particular characteristic to provide an absolutely tranquil bottom casting process without tipping, that is to say the ingot or other mould may remain stationary, and to attain simultaneously the two physical conditions which are incompatible with the ordinary bottom casting methods, namely of obtaining throughout the casting operation a sluggish flow of the liquid current both from the point where the feeding or charging conduit joins the lower part of the mould as well as to the point where the feeding duct receives the poured metal, which is realized by maintaining the level of the molten metal poured into the mould at such a height that it is constantly and substantially the same in the interior of the mould and in the feeding duct, although at each instant the height of the fall between the vessel, or ladle from which the molten metal is poured and the surface of the metal already poured into the duct may be much reduced.

The arrangement employed has also a particular characteristic feature, and that is the feeding conduit, or conduits, is formed proportionally with the operation of filling the mould, by successively assembling, during that operation, the several elements constituting the conduit, elements which are placed one above another as the level of the poured-in metal rises in the mould. The height of the tipping is thus at the most equal to that of one of the elements constituting a conduit.

In the accompanying drawings:

Figs. 1 to 3 are vertical sections of an example of the device for carrying into

effect the process according to the invention, showing three different successive states of the casting operation.

Fig. 4 shows, in vertical section, a device for the molding of large and complicated castings.

Fig. 5 is a vertical section of one of the elements that constitute the lateral conduit or conduits for supplying the molten metal to the mold.

Fig. 6 shows, in vertical section, another example of the device for carrying into effect the process according to the invention, such a device having two lateral supply conduits.

Figs. 7 and 8 represent two modified forms of the device with two lateral conduits.

In Figs. 1 to 3, 1 is a mould, 2 is the orifice where the feeding or charging conduit opens into the mould; 3 is the horizontal portion of this conduit, 4 is part which serves for the initial tipping, 5 is one of the elements constituting the vertical part of the feeding conduit, the element being added at the moment when the level of the poured-in metal approaches the upper portion of the part 4; other analogous elements subsequently added in the same manner are shown at 6, 7 and 8. In the last added element of the pile thus formed the filling terminates, that is at the level 10.

Each element is set in place after the preceding element has been filled, so that the height of the free fall of the metal is, at a maximum, equal to the height of an element.

Fig. 2 represents an intermediate phase and Fig. 3 the final phase of the operation, after which the final filling of the mould can be completed without inconvenience by direct pouring in at the top 11.

Fig. 4 shows, also by way of example, a similar arrangement for filling a sand mould.

It is evident without departing from the characteristics of the present invention that the several elements successively added to form the feeding conduit as expansion of the metal in the mould occurs may be entirely or partly of metal, and be lined with a refractory substance or with sand (Fig. 5), may have any form and section appropriate to the desired end, may consist of one or more removable parts, may be socketed or be simply placed one upon another, be free or be fixed and be arranged in position by hand or by means of any appropriate device.

Horizontal or inclined supplementary conduits such as 12 in Fig. 4 may be interposed as auxiliary elements between the ordinary elements, to permit of filling very high moulds without having to take into account the condition of the metal already cast at the bottom.

A mould can be fed by means of a single group of elements, or several groups of elements constituting several feeding conduits or be united to form one as in Figs. 7 and 8.

The elements of the several conduits may be put in place simultaneously or in turn, to the same level or to different levels (Fig. 6).

The tipping into the several conduits may take place simultaneously or in turn by means of a single vessel or several vessels.

A single supply conduit or several conduits may be common to several moulds.

The ascending casting device may of course be employed in combination with any known ingot or other mould casting processes.

The invention is independent of the apparatus which serves as the molten metal receptacle during the pouring, which receptacle may be a ladle with several spouts or lips or a ladle with several stoppers, or several ladles of any suitable form may be used.

What I claim is:

1. An apparatus for molding metals or alloys comprising a vertical mold and a substantially vertical conduit communicating with the bottom of the mold, said conduit being formed of a plurality of separable sections, whereby said conduit is adapted to be built up step by step, for the purpose described.

2. An apparatus for molding metals or alloys, comprising a mold and a conduit communicating with the bottom thereof and a plurality of conduit sections adapted to be placed in communication with said conduit one above the other, for the purpose described.

3. The process of casting metals or alloys by introducing the molten material into the mold through a conduit communicating with the bottom thereof, which comprises pouring the molten material into the conduit at vertically separated points therein in accordance with the rise in level of the molten material in the mold and conduit.

In testimony whereof I affix my signature.

PIERRE HENRI GASTON DURVILLE.